

May 7, 1935.

R. HOFSTADT

2,000,388

MANUFACTURE OF RIBBONS

Filed Feb. 27, 1932

No. 1 

No. 7 

No. 2 

No. 8 

No. 3 

No. 9 

No. 4 

No. 10 

No. 5 

No. 11 

No. 6 

No. 12



No. 13



Inventor

Richard Hofstadt

By his Attorneys

Byrnes Townsend & Potter

## UNITED STATES PATENT OFFICE

2,000,388

## MANUFACTURE OF RIBBONS

Richard Hofstadt, Wolfen, near Bitterfeld, Germany, assignor to I. G. Farbenindustrie Aktiengesellschaft, Frankfort-on-the-Main, Germany

Application February 27, 1932, Serial No. 595,639  
In Germany March 4, 1931

7 Claims. (Cl. 18—15)

My present invention relates to the manufacture of ribbons and more particularly to the manufacture of ribbons from solutions containing cellulose or derivatives thereof.

5 One of its objects is the nozzles to produce ribbons provided with patterns by the wet-spinning process. Another object is to produce the new ribbons provided with patterns. Further objects will be seen from the detailed specification following hereafter. Reference being had to the accompanying drawing in which

Figs. 1 to 10 represent some forms of the opening of the nozzles used in the spinning process for obtaining ribbons provided with patterns.

15 Fig. 11 shows diagrammatically the cross section of a ribbon provided with patterns according to my invention when, for instance, spun with a nozzle having an opening as represented in Fig. 10.

Fig. 12 instances a cross section of the new ribbons when cut in the dry state, and

20 Fig. 13 instances a part of a cross section of the new ribbons when cut in the wet state.

According to my present invention it is possible to obtain particularly effective ribbons, by 25 spinning from a nozzle whose orifice has the form of a longitudinal main slot having slots branching laterally therefrom. By means of nozzles having such orifices it is possible to produce ribbons which exhibit special effects. These effects consist 30 mainly in patterns having a strike-like appearance which may be regularly or irregularly distributed over one or both faces of the ribbon. Depending upon the length of the lateral branches of the slot of the nozzles there are obtained 35 either narrower or broader stripes. At the places where the layers overlap, the white, undyed ribbon appears less transparent or duller, the dyed one darker.

It is also possible to give the lateral branches 40 and the main slot of the nozzles different breadths and different lengths, thus the lateral branches may be broader than the main slot. In the latter case ribbons may be obtained which are more flexible and by their increased pliability allow 45 easier working up in certain machines. It is also possible to give the lateral slots being positioned near the centre of the main slot a greater length so that the stripes on both faces of the ribbon overlap, whereby a stiffening of the whole ribbon 50 takes place. In the same manner if giving the lateral slots branching off the ends of the main slot a greater length a stiffening of the ends of the ribbon is obtainable. By these means special 55 advantages may be obtained according to the methods of working up the ribbons. Further-

more, the main slot need not be rectilinear; it may be wavy or have any other irregular form.

While spinning the ribbons, the speed of draft must be adapted to the speed with which the spinning solution is squirted into the spinning bath, in order to avoid a strong stretching which would cause a deformation of the ribbons if not yet completely coagulated.

The ribbons, after leaving the bath, are preferably guided over some rods or rollers in order to maintain them infolded during the coagulation, or other treatment until they are fixed on the bobbin or other receiving device.

In spinning through the nozzles according to the present invention there will be produced the 15 proper ribbon by the main slit from which small ribbons branch off formed by the lateral slits. The ribbon can be produced as above explained in a process analogous to the method of spinning on bobbins, however, they may likewise be produced in continuous or any other suitable manner. The ribbons obtainable according to this invention show in the dry state a cross section under the microscope as illustrated in Fig. 12 or diagrammatically illustrated in Fig. 11. It is seen 20 from Fig. 13 that the lateral ribbons, the ribbon consisting in this particular case of cellulose hydrate, form nearly one piece with the main ribbon when wetted so that only a line of separation is 25 seen.

30 The following examples illustrate the invention:

*Example 1.*—By spinning a viscose, containing 7.5 per cent of cellulose and 7 per cent of alkali, at such a speed that 42 cc. of viscose are pressed 35 per minute through the nozzle into the precipitating bath, a ribbon having a strength of 1900 deniers is obtained. The nozzle has a main slot of 13 mm. length and 0.1 mm. breadth from which 6 lateral slots branch off at an angle of 40 about 60°. On each side of the main slot there branch off 3 lateral slots at an equal distance in the manner shown in Fig. 10, each having a length of 2 mm. and a breadth of 0.1 mm.

The spinning bath employed contains 14 per 45 cent of sulfuric acid and 30 per cent of sodium sulfate and is heated to a temperature of about 45° C. The speed of draft is 20 m. per minute. The ribbon produced is preferably guided in a weakly stretched condition, over several glass 50 rods or the like, in order to prevent it from rolling.

A uniformly figured ribbon of 3 to 4 mm. breadth is obtained.

*Example 2.*—The viscose and the spinning conditions are the same as in Example 1. The noz- 55

zle employed has a main slot of 13 mm. length and 0.15 mm. breadth; at the ends of the main slot two lateral slots of 0.15 mm. breadth and 2.5 mm. length branch off at right angles and in 5 the middle part of the main slot a lateral slot of the same size branches off at an angle of 60°. The opening of this nozzle is of the form shown in Fig. 6.

10 An irregularly striped ribbon having reinforced edges of 1900 deniers is obtained.

15 Example 3.—53 cc. of viscose containing 13.8 per cent of cellulose and 7 per cent NaOH are pressed within a minute through the nozzle into the precipitating bath. The nozzle employed has a main slot of 18 mm. length and 0.1 mm. breadth from which there branch off 8 lateral slots at an angle of 60°, each having a length of 1.6 mm. and a breadth of 0.1 mm. The precipitating bath is identical with that of Example 1.

20 There is obtained a uniformly striped ribbon of 4500 deniers and a breadth of 9 to 10 mm.

25 The appearance of the figured ribbon depends upon the speed of draft, the uniform delivery of the spinning solution and the size and arrangement of the slots of the nozzles. These conditions must be well adapted to one another and should be determined by a few preliminary trials.

30 With regard to the viscosity and the maturation of the spinning solution, the same rules are applied as those known for the spinning of viscose silk. They may according to the spinning bath and the spinning conditions, vary within wide limits.

35 The ribbon wound on the spool or unwound therefrom is after-treated in the manner usual for artificial silk, bleached, if desired, and dried.

40 My invention is not limited to the foregoing examples nor to the specific details given therein. Other forms of the openings of the nozzle may be used. Furthermore, the spinning conditions may be varied within wide limits. Other cellulose solutions than viscose may be used as spinning solutions, the methods of spinning are the same as those known from the production of artificial silk and familiar to every chemist skilled in the art provided that the lines given in this specification be observed.

What I claim is:

1. A nozzle for the manufacture of ribbons provided with patterns which has an opening forming a main slot of 13 mm. length and 0.1 mm. breadth from which 6 lateral slots of 2 mm. length and 0.1 mm. breadth branch off at an angle of 60°, 3 of the lateral slots being arranged on each side at equal distances in such manner that the slots positioned at the end of the main slot are inclined towards each other. 5

10 2. A nozzle for the manufacture of ribbons provided with patterns which has an opening forming a main slot of 13 mm. length and 0.15 mm. breadth from which 3 lateral slots of 2.5 mm. length and 0.15 mm. breadth branch off, 2 of these slots branching off opposite sides of the main slot at a right angle, the third lateral slot branching off the middle part of the main slot at an angle of 60° and being inclined to the slot arranged on the other side of the main slot. 20

25 3. Ribbons consisting of cellulose hydrate provided with patterns having a stripe-like appearance, said patterns being formed by partially overlapping layers.

30 4. Ribbons consisting of cellulose hydrate provided with patterns having a stripe-like appearance comprising a main ribbon having attached thereto small ribbons partially overlapping the main ribbon.

35 5. Ribbons consisting of cellulose hydrate provided with patterns having a stripe-like appearance comprising a main ribbon having attached thereto small ribbons partially overlapping the main ribbon and each other.

40 6. Ribbons consisting of cellulose hydrate provided with patterns having a stripe-like appearance comprising a main ribbon having attached to both its ends small ribbons partially overlapping the main ribbon.

45 7. A ribbon consisting of cellulose hydrate provided with patterns having a stripe-like appearance, said patterns constituting a superimposed portion of the material of the ribbon integral therewith.

RICHARD HOFSTADT. 45